

# United States Patent Office

2,699,392

Patented Jan. 11, 1955

1

2,699,392

## VESICULAR PRINTS AND PROCESS OF MAKING SAME

Clifford E. Herrick, Jr., Easton, Pa., and Ann K. Balk, Owego, N. Y., assignors to General Aniline & Film Corporation, New York, N. Y., a corporation of Delaware

No Drawing. Application December 12, 1951,  
Serial No. 261,375

17 Claims. (Cl. 95—7)

This invention relates to a method of preparing a photosensitive vesicular print material by forming a solution in a solvent of a thermoplastic, hydrophobic resin such as cellulose acetate with a resinous copolymer of a vinyl compound such as methyl vinyl ether and an ethenoid dicarboxylic acid compound such as maleic anhydride, coating this solution on to a support such as glass or black paper, drying to make a continuous film, treating the coating with a moist base such as ammonia vapor to make it hydrophilic, applying an aqueous solution of a stabilized photosensitive diazonium compound and drying. The invention also relates to the resulting substantially clear, photosensitive, vesicular print material, to the method of preparing stable vesicular prints therefrom by irradiating with actinic light through a design and then subjecting to elevated temperatures for short times to develop and stabilize the images, as well as to the resulting stable vesicular prints.

The art is familiar with photographic vesicular images prepared from a light sensitive layer made up from a hydrophilic material such as gelatin and a photosensitive diazo compound which liberates nitrogen gas upon photo-decomposition. The image is developed by treatment with steam or water, whereby the hydrophilic layer softens and the nitrogen gas therein expands forming minute vesicles which refract light which strikes the layer. This causes an appearance of whiteness by reflected light and darkness by transmitted light. Sometimes the resulting print is given a treatment with a coupling compound to render the unexposed diazo material non-photosensitive, to prevent subsequent undesirable bubble formation in the unexposed or clear areas upon subsequent overall exposure to ordinary light and moisture.

Many disadvantages are inherent in this process and the resulting prints. The development operation is cumbersome and critical, and gives strong relief effects which are undesirable in photographic prints. In the treatment of the undecomposed diazo material with a coupling component an azo dye is formed, and this prohibits the use of foil vesicular prints as photographic negatives; furthermore, the white areas are badly colored thereby.

A particularly disadvantageous feature thereof is the instability of the vesicular prints in the presence of moisture; since the hydrophilic medium absorbs moisture and softens, the minute vesicles collapse and the image is lost.

An improvement in this vesicular print process is the use of a single application of heat in the development step, giving clean whites, and improved tone gradation through the use of a non-reflecting, opaque backing for positive prints. However, even these improved prints leave much to be desired from the viewpoint of stability toward moisture.

It has been found, in accordance with the invention, that the above discussed drawbacks may be overcome and superior vesicular print materials may be prepared by forming a solvent solution of 5 to 1 parts by weight of a thermoplastic, hydrophobic resin and 1 to 6 parts of a compatible resinous copolymer of about one mol of a vinyl compound with about one mol of an ethenoid dicarboxylic acid compound, coating it on a support and drying to form a continuous layer, treating the layer with a moist base to make it hydrophilic, then sensitizing this layer by application of an aqueous solution of a stabilized photosensitive diazonium compound, prefer-

2

ably including an acidic diazo stabilizer and a plasticizer, and drying. Upon irradiating the resulting material with actinic light through a design, and then subjecting it to an elevated temperature for a short time, the image is developed and the water sensitivity of the layer is greatly reduced. If desired, the resulting vesicular print may be re-exposed to the actinic or ultraviolet light at ambient temperatures to destroy remaining diazo compound.

The resulting vesicular prints are stable at ambient temperatures even in the presence of moisture, exhibiting perfectly clean whites with no discoloration in exposed or unexposed areas. They show no grain and have very soft tone gradation with details in both highlight and shadow areas.

15 The objects achieved in accordance with the invention as described herein include the provision of vesicular images with excellent tone gradation and clean whites; the provision of vesicular prints which show good stability to actinic light, moisture and water at ambient temperatures; 20 the provision of processes for making either positive or negative vesicular prints having the above-mentioned characteristics; the provision of a photosensitive vesicular print layer which is hydrophilic and gas impermeable during the irradiation but which becomes much more hydrophobic during the elevated temperature development treatment; the provision of methods for preparing photosensitive vesicular print materials by forming solvent solutions of thermoplastic hydrophobic resins and compatible resinous copolymers of a vinyl compound with an ethenoid 25 dicarboxylic acid compound, coating this on a support, drying, treating with a moist base, applying an aqueous solution of a stabilized photosensitive diazonium compound and drying; and other objects which will become 30 apparent as details or embodiments of the invention are set forth hereinafter.

In order to facilitate a clear understanding of the invention, the following preferred specific embodiments are described in detail:

### Example 1

A coating formulation was prepared from the following:

12 parts vinyl methyl ether and maleic anhydride copolymer (parts are by weight)  
6 parts cellulose acetate  
19 parts ethylene glycol mono methyl ether  
112 parts acetone  
2 parts polyvinyl methyl ether (plasticizer)

The solids were well dispersed in the liquids and the entire mixture was rolled for several hours to dissolve. The solution was coated on black paper at 25 mils wet film thickness with a Bird type or other applicator, and dried. The layer was passed through ammonia vapors several times (for a total contact time of 3/4 minute at 180° F.), then washed with dilute HCl (e. g., 2 cc. 37% HCl added to 100 cc. of water), dried at 50° C., and sensitized by immersion in the following solution:

10 parts N,N-diethylaniline, 4-diazonium chloride, zinc chloride double salt  
60 10 parts citric acid  
8 parts ethanol  
17 parts ethylene glycol. Entire solution is diluted to about 100 parts with water.

65 The dried layer was exposed to ultraviolet rays through a suitable positive transparency for 30 seconds to about 3 minutes, depending upon the strength of the light source, and developed by the sudden application of heat, as in a rotary ironing mangle (at a temperature of about 190° F. and a contact time of about 5-6 seconds); and a stable image was formed, possessing excellent whites, soft gradation, and good resistance to moisture at ambient temperatures. A brief re-exposure to direct actinic light at ambient temperatures destroys the remaining diazo compound without adversely affecting the prints.

### Example 2

In this example the procedure was as in Example 1, except that the following coating formulation was used:

80 12.66 parts vinyl methyl ether, maleic anhydride copolymer

6.33 parts cellulose acetate  
19.0 parts ethylene glycol mono methyl ether  
112.0 parts acetone  
1.0 part polyvinyl methyl ether

The product gave prints comparable to those in Example 1, by the above-described method.

*Example 3*

In this example the procedure was as in Example 1, except that the following coating formulation was used:  
3.0 parts vinyl methyl ether, maleic anhydride copolymer  
6.5 parts cellulose acetate  
9.5 parts ethylene glycol mono methyl ether  
57.0 parts acetone  
0.50 part polyvinyl methyl ether

The product gave prints similar to those in Example 1, by the above-described method.

*Example 4*

In this example the procedure was as in Example 1, except that the coating was at 18 mils thickness, and the following coating formulation and sensitizing solution were used:

**Coating formulation:**  
6.66 parts vinyl methyl ether, maleic anhydride copolymer  
3.33 parts cellulose acetate  
9.5 parts ethylene glycol mono methyl ether  
57.0 parts acetone  
0.5 part triphenyl phosphate  
0.5 part methyl phthalyl ethyl glycolate

**Sensitizing solution:**  
10 parts N,N-diethyl aniline, 4-diazonium chloride, zinc chloride double salt  
10 parts citric acid  
12.6 parts glycerine. Solution is diluted to about 100 parts with water.

Following the procedure in Example 1, the resulting materials gave prints of good quality and resistance to moisture at ambient temperatures.

*Example 5*

In this example the procedure was as in Example 1, except that the coating was at 18 mils thickness, and the following coating formulation was used:

1.5 parts 2-methoxy-ethyl vinyl ether, maleic anhydride copolymer  
3.5 parts polyvinyl acetate  
28 parts acetone  
5 parts ethylene glycol mono methyl ether

Following the procedure in Example 1, the resulting materials gave prints, and these showed resistance to moisture at ambient temperatures.

In any of these examples, a softer shadow gradation can be obtained by subjecting the print material to a uniform pre-exposure amounting to about 1 to 5% of the exposure required beneath the design.

*Example 6*

The procedure used in this example was the same as in Example 5, except that the following coating formulation was used:

1.5 parts vinyl isobutyl ether, maleic anhydride copolymer  
3.5 parts nitro cellulose  
28 parts acetone  
5 parts ethylene glycol mono methyl ether

Following the procedure in Example 1, the resulting materials gave prints, and these showed resistance to moisture at ambient temperatures.

*Example 7*

The procedure used in this example is the same as in Example 5, except that the following coating formulation is used:

3.0 parts vinyl methyl ether, maleic anhydride copolymer  
7.0 parts methyl methacrylate, polymerized  
57.0 parts acetone  
9.5 parts ethylene glycol mono methyl ether

The vesicular print material is processed as in Example 1.

*Example 8*

The procedure used in this example was the same as in Example 5, except that the following coating formulation was used:

1.5 parts vinyl isobutyl ether, maleic anhydride copolymer  
3.5 parts polyvinyl acetate  
31.0 parts butyl acetate  
5.0 parts ethylene glycol mono methyl ether

The vesicular print material was processed as in Example 1.

*Example 9*

The procedure used in this example was the same as in Example 5, except that the following coating formulation was used:

3.33 parts 2-methoxy ethyl vinyl ether, maleic anhydride copolymer  
6.66 parts cellulose acetate  
57 parts acetone  
9.5 parts ethylene glycol mono methyl ether

Following the procedure in Example 1, the resulting materials gave prints of superior resistance to moisture at ambient temperatures.

*Example 10*

The procedure used in this example was the same as in Example 5, except that the following coating formulation was used:

3.33 parts 2-ethoxy ethyl vinyl ether, maleic anhydride copolymer  
6.66 parts cellulose acetate  
57 parts acetone  
9.5 parts ethylene glycol mono methyl ether

Following the procedure in Example 1, comparable results were obtained.

Comparable results to the foregoing are achieved by using the following variations: Instead of the black paper, a transparent support such as glass, cellophane, or other suitable transparent material may be used to give a negative print; or alternatively, an opaque material such as metal or the like may be used to give a positive print. The opaque material may be of any color, as desired. Where indicated, an intermediate adhesive layer may be used. Instead of treating with ammonia vapors, moist vapors of another volatile base such as organic amines and the like may be used; or alternatively, an aqueous solution of a basic material may be used to render the layer hydrophilic. The thermoplastic hydrophobic resin may be any such resin or mixture of resins which is compatible with the copolymer material providing it remains essentially hydrophobic under the treatment by which the copolymer material is rendered hydrophilic. Copolymers of vinyl compounds with ethenoid dicarboxylic acid compounds are known. In general they are thermoplastic solids and are made up from a ratio of about one mol of the vinyl compound with about one mol of the ethenoid dicarboxylic acid compound; the latter may be maleic anhydride or a substituted maleic anhydride such as one containing a lower alkyl group or the like. Mixtures of resins may be used, as may mixtures of the ethenoid compounds.

The proportions of resin and copolymer should be such as to give compatible compositions when dried, i. e., give a substantially clear layer or film.

Desirable light sensitive diazonium compounds are stabilized as diazo oxide or as the zinc chloride, or the like, metallic double salt and are derived from aromatic para-diamines, particularly N-mono or di-substituted benzene para-diamines or from para-amino diphenyl amine; and 4-diethylamino benzene diazonium chloride is preferred. Diazonium derivatives of naphthols are also suitable.

Other acidic stabilizers may be used, such as lower carboxylic acids, especially hydroxy carboxylic acids. Also, other plasticizers may be used. If desired, thiourea or the like material may be included with the diazo material.

The heating or development step is preferably carried out by direct contact with a heated surface. However, other heating means, such as radiant heat may be used. For some applications, where water resistance is not critical, direct steam may be used.

It is indeed surprising that the processes of the invention may be carried out in a most practical manner, and

yet give vesicular prints which combine good photographic quality with a high degree of stability.

Variations and modifications of the invention will be apparent to one skilled in the art in view of the foregoing disclosures, and it is intended to include within the invention all such modifications and variations except as do not come within the scope of the appended claims.

We claim:

1. A method of preparing a photosensitive vesicular print material which comprises forming a compatible solvent solution of an amount in the range of 5 to 1 parts by weight of a thermoplastic, hydrophobic resin selected from the group consisting of cellulose acetate, nitrocellulose, polyvinyl acetate and polymethyl methacrylate, and an amount in the range of 1 to 6 parts of a resinous copolymer of about one mol of a vinyl ether with about one mol of a maleic acid compound, said hydrophobic resin and said copolymer being compatible, said amounts being selected to give a substantially clear layer upon drying, coating it on a support and drying to form a substantially clear layer, treating said layer with a moist water soluble nitrogenous base to make it hydrophilic, photosensitizing this layer by application of an aqueous solution of a stabilized photosensitive diazonium compound, and drying.

2. The method of claim 1 wherein the maleic acid compound is maleic anhydride.

3. The method of claim 1 wherein the resin is cellulose acetate and the copolymer is of a vinyl ether and maleic anhydride.

4. The method of claim 3 wherein the diazonium compound is N,N-diethylaniline-4-diazonium chloride, zinc chloride double salt.

5. The method of claim 4 wherein the ether is methyl vinyl.

6. The method of claim 4 wherein the ether is 2-methoxyethyl vinyl.

7. The method of claim 4 wherein the ether is 2-ethoxyethyl vinyl.

8. The method of claim 1 wherein the resin is polyvinyl acetate and the copolymer is of a vinyl ether and maleic anhydride.

9. The method of claim 8 wherein the diazonium compound is N,N-diethylaniline-4-diazonium chloride, zinc chloride double salt.

10. The method of claim 9 wherein the ether is isobutyl vinyl.

11. The method of claim 9 wherein the ether is 2-methoxyethyl vinyl.

12. The method of preparing a stable vesicular print which comprises irradiating with actinic light through a design, a photosensitive print prepared according to the method of claim 1 to form a latent image, and then heating said material to develop and stabilize the image.

13. A photosensitive vesicular print material prepared according to the method of claim 1.

14. A photosensitive vesicular print material prepared according to the method of claim 2.

20 15. A photosensitive vesicular print material prepared according to the method of claim 3.

16. A photosensitive vesicular print material prepared according to the method of claim 4.

25 17. A photosensitive vesicular print material prepared according to the method of claim 5.

#### References Cited in the file of this patent

##### UNITED STATES PATENTS

|    |           |               |               |
|----|-----------|---------------|---------------|
| 30 | 2,156,069 | Schlack ----- | Apr. 25, 1939 |
|    | 2,239,704 | De Boer ----- | Apr. 29, 1941 |
|    | 2,397,866 | McQueen ----- | Apr. 2, 1946  |

##### FOREIGN PATENTS

|    |         |                     |               |
|----|---------|---------------------|---------------|
| 35 | 318,511 | Great Britain ----- | Aug. 7, 1930  |
|    | 402,737 | Great Britain ----- | Mar. 5, 1932  |
|    | 524,786 | Great Britain ----- | Aug. 14, 1940 |
|    | 563,804 | Great Britain ----- | Aug. 30, 1944 |